

Feb. 22, 1927.

1,618,515

W. C. CORYELL

METAL WORKING

Filed May 28, 1921



FIG. 2.



FIG. 1.



FIG. 4.



FIG. 3.

INVENTOR

W. C. Coryell.

## UNITED STATES PATENT OFFICE.

WILLIAM C. CORYELL, OF YOUNGSTOWN, OHIO.

## METAL WORKING.

Application filed May 28, 1921. Serial No. 473,477.

- The present invention relates to the art of metal working and consists essentially in working the metal by subjecting the same to a high compression while it is under a high tension. More particularly the working consists of reducing the thickness or sectional area and of elongating the length of the piece by a combined pulling and compressing means.
- 10 I have found that the pulling of a piece of steel at a high tension, for example at near its elastic limit, while compressing it between rolls at about its crushing strength there is produced very much more fluidity in the metal and at the same time much less hardening effects on the steel due to rolling. This permits the rolling to be carried on to a very much greater extent than where only compression between the rolls is employed, 20 as in present practice.
- In the old method of cold rolling of low carbon steel, by simply passing it between the rolls, an elongation of from 25% to 50% is about all that the steel will withstand 25 without reannealing. Somewhat greater elongations can be made, especially if the steel is a low carbon steel and if small diameters of rolls are used. The effect of the latter is to produce an excessive elongation for 30 each passage of the metal through the rolls.
- According to my new method of combined pulling and compressing, very much greater elongations are obtainable in a given carbon and anneal of the steel, without the necessity 35 of reannealing. Thus as demonstrated by me, when a high tension is in one direction and a large compression is at substantially right angles thereto there is produced a greater resultant force within the steel which 40 produces a very much greater fluidity of the metal. Under such conditions I have obtained elongations of from 1000% to 1200% and the material does not appear to be in any greater need of reannealing than 45 did steels which were elongated from 25% to 50% or possibly 100% by the old non-pulling method.
- In the accompanying drawing, Fig. 1, I have illustrated my invention diagrammatically representing the pulling of the piece 50 after passing the rolls. Figure 2 represents a tension in the piece produced by a pull at each end. Figure 3 shows the rolling of a hoop or steel belt. Figure 4 shows a simple diagram of two equal forces at right angles and their resultant force. In these diagrams, 10 designates a piece of metal passing between rolls 11 and 12 and having its end or ends engaged by a gripping and tensioning device 13. As soon as the forward end of the piece 10 is passed beyond the rolls 11 and 12, the device 13 is attached to it. The necessary tension is then given to the steel by pulling on the device 13, as indicated by the adjacent arrow 14. The amount of pull, as before noted, should be very great approximating for example, the elastic limit of the metal. A heavy compression is applied to the metal of the rolls 11 and 12. These rolls are driven as usual and are 70 pressed toward each other, as indicated by the opposed arrows 15, by any suitable compressing means, such as a screwdown, examples of which will be found in my prior United States Patents No. 1,211,029, granted April 3rd, 1917, and No. 1,233,647, granted July 17th, 1917. The amount of compression, as before noted is in the neighborhood of the crushing strength or elastic limit of the metal of the strip 10, or a slightly 80 greater pressure may be used.
- Under certain conditions, we may apply the high tensional force to the piece on the entering side of the mill and in other cases to only the outgoing side of the mill. When 85 the pull is applied to only the outgoing end, there is a tendency for the material to accumulate in front of the rolls, as at 16, as a sort of bulge or double wave. But when a pull is exerted on the ingoing end as in Figures 2 or 3, this wave does not appear, as at 90 17. The disappearance of this wave is of assistance in accomplishing great elongations. In cold rolling, 16 and 17 are usually 95 not apparent to the eye, but the tendency exists, nevertheless.
- The figures represent the forces of tension and compression as being approximately equal. In actual practice they are not required to be equal. There is no well defined stress in the compression or tension applied at which the greater fluidity begins or ends. If the material is of much value as is a steel belt, I recommend keeping the

pull safely below the elastic limit and increasing the compression to such a point as to produce the desired fluidity in the reduction. If rapid reduction or great production is desired, a pull can be exerted closer to the elastic limit or even exceeding it.

In the old method, the flow occurs under the sole impulse of the compressive force of the rolls while in my method there are two more or less equal forces acting simultaneously at right angles to each other, the resultant of which forces is roughly 40% greater than either of the components, when they are equal. When they are unequal, the resultant is less than 40% greater than the maximum of the two forces.

The metal 10 may be rolled when either hot or cold and may be presented in any shape, such as a belt, band, sheet, strip, bar, tube, wire, rod or the like. It, of course, may be any malleable or ductile metal.

In the diagram of forces of Fig. 4, the horizontal line "a b" represents the tensional force pulling in the direction of the arrow 14, the line "c a" represents the compressing force acting in the direction of the arrow 15, and the line "c b" represents the resultant force. As here shown, the two component forces are equal and the resultant force in this case is, roughly, 40% greater. These relative values are here shown by the numerals 1, 1 and 1.4 upon the diagram. Obviously with slight changes in the direction or magnitude of the components, changes would be produced in the resultant. This diagram does not contemplate the secondary forces which are acting in my process. Although I have used the word "fluidity" in several instances throughout this description, it may be that such words as "ductility" or "plasticity" would more correctly define the action or condition of the metal. This might be further explained by reference to the art of malleation wherein metals are worked down to extreme thinness by a hammer or by means of rolls. In that aspect of the present invention, the force exerted on the metal blank by the pressure of the rolls is a malleating force which is superior to the resistance of the metal, causing the latter to flow and spread and thereby be reduced in thickness. Simultaneously, in fact exactly coincident therewith, another force is applied to the metal blank at the time the malleating pressure is imposed thereon, namely, an elongating force which is exerted preferably in a direction at right angles to the line of force of the rolls. The resultant of these two forces within the body of the metal is greater than either of said forces singly and is also greater than the elastic limit of the metal with the result of obtaining the deformation of the metal in the manner contemplated. This important phase of the invention distinguishes from

prior suggested practices wherein a mere tension is maintained on the metal while it is being rolled, simply to keep it in form. It should be borne in mind that the present invention is also applicable to the working of other materials than metal.

What I claim as new and desire to secure by Letters Patent of the United States, is—

1. The method of working a ferrous metal piece, which includes the operations of pressing the piece between rolls applying a force approaching the elastic limit of the metal, and simultaneously drawing out the advancing portion of the piece beyond the rolls with a tensional force approaching the elastic limit of the metal.

2. The method of working ferrous metal which includes the operations of pulling the metal longitudinally throughout its whole length at about its elastic limit and at the same time compressing the same transversely throughout its whole thickness at about its elastic limit, the two forces being applied simultaneously and the compressive force being applied progressively throughout the length of the metal.

3. The method of working metal which includes the combined operations of pulling an endless piece of metal throughout its whole length and compressing the metal progressively, each force being applied at about the elastic limit of the metal and both forces being effective at a common point.

4. The method of greatly extending the length and greatly reducing the thickness of a piece of ferrous metal by subjecting the same, one transverse portion after another in succession, simultaneously to a compressive stress and a tensile stress, each stress being at about the elastic limit of the metal and each acting upon every point in the successive cross sections worked upon, whereby all parts of the metal piece, except possibly the ends, are subject at one time or another to the resultant of both said stresses.

5. The method of greatly extending the length and greatly reducing the sectional area of a piece of ferrous metal, by subjecting the transverse portion of the metal simultaneously to a compressive stress between reducing rolls and to the tensile stress applied by a pulling device over which said piece has been looped, each stress being at about the elastic limit of the metal and being applied progressively, simultaneously each with the other, along the length of the piece.

6. The method of elongating a piece of metal to more than five times its original length without reannealing the piece, which method consists in simultaneously applying to the piece successively from point to point along its length tensional and compressional forces each in the neighborhood of the elastic limit of the metal directed at an angle to

each other so that the resultant force within the metal has a greater value than either of said component forces.

7. The method of progressively rolling an endless strip by passing it round and round through a pass between rolls and applying tension to the length of the strip, the com-

pressive stress exerted by the rolls and the tensile stress both approaching the respective elastic limits of the metal.

10

In testimony whereof, I hereunto subscribe my name this 25th day of May A. D. 1921.

WILLIAM C. CORYELL.

each other so that the resultant force within the metal has a greater value than either of said component forces.

7. The method of progressively rolling an endless strip by passing it round and round through a pass between rolls and applying tension to the length of the strip, the com-

pressive stress exerted by the rolls and the tensile stress both approaching the respective elastic limits of the metal.

In testimony whereof, I hereunto subscribe my name this 25th day of May A. D. 1921.

WILLIAM C. CORYELL.

10

### DISCLAIMER

1,618,515.—*William C. Coryell, Youngstown, Ohio. METAL WORKING. Patent dated February 22, 1927. Disclaimer filed December 11, 1934, by the assignees, United Engineering & Foundry Company and American Sheet & Tin Plate Company.*

Hereby disclaim from said specification that part thereof appearing in lines 17 and 18 of page 2, reading as follows: "when either hot or".

And your petitioners further hereby disclaim from said specification that part thereof appearing in lines 19, 20 and 21 of page 2, reading as follows: "bar, tube, wire, rod or the like. It, of course, may be any malleable or ductile metal."

And your petitioners further hereby disclaim from said specification that part thereof appearing in lines 68, 69, 70, and 71 of page 2, reading as follows:

"It should be borne in mind that the present invention is also applicable to the working of other materials than metal."

And your petitioners further hereby disclaim from the scope of each of claims 1 to 6, inclusive, all material except ferrous metal belts, bands, sheets and strips, and all ferrous metal belts, bands, sheets and strips not having a width materially greater than that of flat wire.

[Official Gazette January 1, 1935.]

## DISCLAIMER

1,618,515.—*William C. Coryell*, Youngstown, Ohio. METAL WORKING. Patent dated February 22, 1927. Disclaimer filed December 11, 1934, by the assignees, *United Engineering & Foundry Company* and *American Sheet & Tin Plate Company*.

Hereby disclaim from said specification that part thereof appearing in lines 17 and 18 of page 2, reading as follows:

“when either hot or”.

And your petitioners further hereby disclaim from said specification that part thereof appearing in lines 19, 20 and 21 of page 2, reading as follows:

“bar, tube, wire, rod or the like. It, of course, may be any malleable or ductile metal.”

And your petitioners further hereby disclaim from said specification that part thereof appearing in lines 68, 69, 70, and 71 of page 2, reading as follows:

“It should be borne in mind that the present invention is also applicable to the working of other materials than metal.”

And your petitioners further hereby disclaim from the scope of each of claims 1 to 6, inclusive, all material except ferrous metal belts, bands, sheets and strips, and all ferrous metal belts, bands, sheets and strips not having a width materially greater than that of flat wire.

[*Official Gazette January 1, 1935.*]